

Nov. 4, 1958

J. T. MARSH ET AL  
PROCESS FOR THE TREATMENT OF FABRICS WITH  
RESINOUS CONDENSATION PRODUCTS

2,859,136

Filed Aug. 22, 1955

2 Sheets-Sheet 1



FIG. 1

J. T. Marsh and  
R. G. Thompson  
Inventors

By  
Marshall, Portee, Miller & Stewart  
Attorneys

Nov. 4, 1958

J. T. MARSH ET AL

2,859,136

PROCESS FOR THE TREATMENT OF FABRICS WITH  
RESINOUS CONDENSATION PRODUCTS

Filed Aug. 22, 1955

2 Sheets-Sheet 2



*J. T. Marsh and  
R. A. Thompson*  
Inventors

*By  
Mason, Porter, Miller & Stewart  
Attorneys*

# United States Patent Office

2,859,136

Patented Nov. 4, 1958

1

2,859,136

## PROCESS FOR THE TREATMENT OF FABRICS WITH RESINOUS CONDENSATION PRODUCTS

John Thompson Marsh, Hale, and Ronald Arthur Blease, Ruislip, England, assignors to Tootal Broadhurst Lee Company Limited, Manchester, England, a British company

Application August 22, 1955, Serial No. 529,774

Claims priority, application Great Britain July 8, 1950

9 Claims. (Cl. 117—145)

This invention which is a continuation-in-part of the now abandoned applications Serial Nos. 235,015, filed July 3, 1951; 295,361, filed June 24, 1952 and 295,362, filed June 24, 1952, relates to improvements in making resin containing textile fabrics composed wholly or mainly of regenerated cellulose.

It is known that many of the properties of textile fabrics are improved when they contain synthetic resins, for example urea-formaldehyde, which have been insolubilised therein. For example textile fabrics composed wholly or partly of cellulose may be rendered crease-resistant or given permanent mechanical effects, improved fastness of many dyestuffs or dimensional stability.

In all these processes heating is used to insolubilise the resin. When a urea-formaldehyde resin is insolubilised by heating in the fibres of a textile fabric composed wholly or partly of cellulose, there is a loss in resistance to abrasion. Accordingly, when the treated fabric is subjected to rubbing, it shows wear more readily than the untreated fabric. This loss in resistance to abrasion is particularly great in the case of fabrics which are composed wholly or mainly of regenerated cellulose. In the past this reduction in resistance to abrasion has had to be tolerated but the fact that the resistance to abrasion has been reduced has meant that large quantities of resin could not usefully be introduced into the fabrics. Even the introduction of quantities sufficient to give crease-resistance causes a serious reduction in the resistance to abrasion. It has therefore been necessary in all cases to accept a compromise between the improvements effected by the resin and the loss in abrasion resistance. In cases where abrasion resistance was a particularly important consideration small quantities of resin have had to be used with consequent sacrifice of some of the desired improvements in physical properties.

It is accordingly an object of the present invention to give increased abrasion resistance to textile fabrics composed wholly or mainly of regenerated cellulose, and having amino-formaldehyde resin insolubilised in the fibres thereof by heating. It is a further object of the invention to enable large quantities of amino-formaldehyde resin to be insolubilised by heating in the fibres of a fabric composed wholly or mainly of regenerated cellulose, without undue loss in resistance to abrasion. It is a still further object of the invention to give increased abrasion resistance to textile fabrics composed wholly or mainly of regenerated cellulose, and having insolubilised by heating in the fibres thereof, a melamine-formaldehyde resin or mixed melamine-formaldehyde urea-formaldehyde resin. These and other objects of the invention will be more apparent from the following description.

The customary method of insolubilising a thermohardening synthetic resin in the fibres of a textile fabric is to impregnate the fabric with an aqueous solution containing the resin-forming ingredients or an intermediate condensation product thereof and an acidic catalyst and thereafter to dry the impregnated fabric and heat it to

2

a temperature of 120–180° C. for a sufficient time to insolubilise the resin, the time and temperature of such heating being inter-related and being chosen in accordance with the activity of the particular acidic catalyst employed. One proposal which has been made to reduce the loss in abrasion resistance is to omit the catalyst from the impregnating mixture and then to supply the catalyst as a steam-volatile organic acid by conducting the final heating in steam box containing an excess of such steam-volatile organic acid. We have found that this procedure gives resins which still have a substantial solubility in water i. e. the resin is not effectively insolubilised in the fabric. Accordingly the effects produced by the resin are not fast to washing.

10 We have found that the loss in resistance to abrasion which accompanies the insolubilisation in a cellulosic fabric of an amino-formaldehyde resin can be materially reduced, without corresponding sacrifice of the desirable properties conferred by the resin, if the final heating to insolubilise the resin is effected in an atmosphere containing a substantial proportion of superheated steam.

15 The use of small quantities of steam in the atmosphere used for heating textile fabrics containing resin-forming ingredients is quite customary and has been recommended in processes for rendering cellulosic fabrics crease-resistant. In fact, the presence of steam can never be altogether avoided since a very small amount of water is liberated during the condensation of the resin. Such an amount of water is quite insignificant and cannot produce in the 20 heating chamber more than a very minute proportion of steam. Proposals have been made to introduce steam into the heating chamber but the customary heating chambers are not capable, without modification, of maintaining, during the heating of a textile fabric, an atmosphere having more than 20% of steam. It might have been 25 thought that when steam was passed into such a chamber at a sufficient rate to be seen escaping from all the openings such heating chamber must contain an atmosphere consisting substantially wholly of steam. Measurements which have been made by the method and apparatus hereinafter to be described show that this is not the case. They 30 show, in fact, that when a textile fabric is passed through a cloth baking machine of the type normally used in the crease-resistant process to which at the same time steam is admitted from a supply at 40 lbs. per square inch pressure until steam is issuing from all the openings in the baking chamber, the atmosphere in the chamber contains much less than 20% of steam. The most careful 35 precautions against steam losses must be taken to maintain in a cloth baking machine of the type normally used, during the heating of a textile fabric, an atmosphere having more than 20% of steam. It might have been 40 thought that when steam was passed into such a chamber at a sufficient rate to be seen escaping from all the openings such heating chamber must contain an atmosphere consisting substantially wholly of steam. Measurements which have been made by the method and apparatus hereinafter to be described show that this is not the case. They 45 show, in fact, that when a textile fabric is passed through a cloth baking machine of the type normally used, during the heating of a textile fabric, an atmosphere having more than 20% of steam. It might have been 50 thought that when steam was passed into such a chamber at a sufficient rate to be seen escaping from all the openings such heating chamber must contain an atmosphere consisting substantially wholly of steam. Measurements which have been made by the method and apparatus hereinafter to be described show that this is not the case. They 55 show, in fact, that when a textile fabric is passed through a cloth baking machine of the type normally used, during the heating of a textile fabric, an atmosphere having more than 20% of steam. It might have been

To secure the objects of the present invention, it is essential that the atmosphere in which the final heating to insolubilise the resin is effected shall contain at least 50% of steam and that this steam be superheated steam. By 60 "superheated steam" we mean steam above the temperature at which it can exist in equilibrium with water at the pressure used for insolubilising the resin. We prefer to work at substantially atmospheric pressure. At atmospheric pressure steam is, of course, superheated at all temperatures above its boiling point.

All the steam percentages given herein refer to the partial pressure of steam expressed as a percentage of the total pressure of air and steam, measured at substantially the temperature of the heating chamber.

The principle of the invention is illustrated in the accompanying drawings in which

Fig. 1 is a graphic representation of the comparison

of the results of the process with oven dry curing and Fig. 2 is a vertical cross-sectional view of the testing apparatus used.

In order to measure the steam content of the chamber in which the textile material is heated the following method may be employed: A sample of the atmosphere of the heating chamber (oven) is withdrawn, the steam condensed therefrom and the proportion of residual air measured.

This can conveniently be done with the aid of the apparatus diagrammatically shown in Figure 2 of the accompanying drawing, as follows:

The flask 1, the volume of which is small compared with the oven, and which is surrounded by a removable heating jacket 2, is connected by a tube 3 having a valve 4 to the oven (not shown), by a tube 5 having a valve 6 to a vacuum pump (not shown) and by a tube 7 to a mercury manometer or to a Bourdon gauge (not shown). The flask 1 is provided with a thermometer 8. The flask 1 is exhausted by the vacuum pump, the valve 6 being open and the valve 4 closed and then brought to the same temperature as the oven. When the flask 1 has been evacuated, as shown by the manometer or the Bourdon gauge, and is at the temperature of the oven, valve 6 is shut and the valve 4 opened for a few seconds to allow a sample of the oven atmosphere to pass into the flask 1. As soon as the pressures are equalised, as shown by the manometer or the Bourdon gauge (the oven is at atmospheric pressure), the valve 4 is closed thus leaving the flask connected only to the manometer or the Bourdon gauge.

The heating jacket 2 is then removed and the flask 1 cooled down to room temperature. As a result of this cooling, the water vapour condenses on the sides of the flask 1 and the cooling of the residual air also leads to a reduction in pressure. The final pressure in the flask 1 is read off on the manometer or the Bourdon gauge, and a knowledge of this and of the initial and final temperatures enables one to calculate the steam content as in the following calculation.

Atmospheric pressure = 760 mm.  
Initial temperature of flask (equals temperature of oven) = 150° C.

Final temperature of flask = 20° C.

Final pressure difference recorded on manometer = 500 mm.

Final pressure in flask = 760 - 500 = 260 mm.

Vapour pressure of water at 20° C. = 17.5 mm.

Therefore, pressure of residual air at 20° C. = 260 - 17.5 = 242.5 mm.

Therefore,

$$\text{Pressure of air at } 150^\circ \text{ C.} = 242.5 \times \frac{423}{293} = 350 \text{ mm.}$$

Therefore, pressure of steam at 150° C. = 760 - 350 = 410 mm.

Therefore,

$$\text{Percent of steam in original sample} = \frac{410}{760} = 54\%.$$

The importance of employing at least 50% of superheated steam in the atmosphere in which the heating to insolubilise the resin is effected is illustrated by the following Table I and the graph shown in Figure 1 of the accompanying drawing. Table I shows the result of a series of tests in which different portions of the same fabric composed wholly of viscose spun rayon were impregnated with the same aqueous solution of urea-formaldehyde condensation product according to the method described in Example 1 but heated in atmospheres containing different proportions of steam. The table shows the percentage improvement in abrasion resistance (ring-wear) of each portion of fabric as compared with a portion heated in an atmosphere not containing steam (dry cure). The abrasion resistance referred to in some of the following tables and elsewhere herein as "ring-

wear" was measured on the "ringwear testing machine" described in the Journal of the Textile Institute, 1935, 26, 93P.

Table I

| Percent Steam | Percent Improvement in Ringwear over dry cure | Percent Steam | Percent Improvement in Ringwear over dry cure |
|---------------|-----------------------------------------------|---------------|-----------------------------------------------|
| 14.1          | 9.5                                           | 58.6          | 68.5                                          |
| 17.4          | -1.0                                          | 59.2          | 38.5                                          |
| 23.0          | 3.0                                           | 60.8          | 74.0                                          |
| 25.0          | 2.0                                           | 63.9          | 81.0                                          |
| 25.0          | -2.5                                          | 65.6          | 70.0                                          |
| 30.0          | -7.0                                          | 69.0          | 46.5                                          |
| 35.5          | 13.0                                          | 69.8          | 58.0                                          |
| 42.2          | 46.5                                          | 70.2          | 51.0                                          |
| 43.9          | 92.0                                          | 72.7          | 86.0                                          |
| 47.0          | 19.0                                          | 77.9          | 96.0                                          |
| 47.8          | 52.0                                          | 80.7          | 61.0                                          |
| 48.8          | 65.0                                          | 81.5          | 66.0                                          |
| 49.1          | 37.0                                          | 83.8          | 89.0                                          |
| 49.7          | 37.0                                          | 84.4          | 88.5                                          |
| 49.7          | 20.0                                          | 86.2          | 123.0                                         |
| 55.2          | 62.0                                          | 91.2          | 86.0                                          |
| 57.3          | 62.0                                          | 92.2          | 108.0                                         |

The figures shown in Table I are represented as crosses on the graph of Figure 1 of the drawing. The crosses occupy positions in a narrow band sloping upwardly to the right and the smooth curve in the middle of the band gives a representation of the improvement in abrasion resistance resulting from increasing the proportion of superheated steam in the atmosphere used for heating. It will be seen that the improvement is particularly striking when the atmosphere contains at least 50% of steam and that in no case where the proportion of steam exceeded 50% was the improvement less than 38.5%.

Accordingly, the objects of the present invention are secured by a process which comprises impregnating the textile fabric with an aqueous solution of water-soluble amino-formaldehyde resin-forming ingredients containing an acidic catalyst for the resin-formation, drying the fabric and heating it to produce water-insoluble thermohardened synthetic resin from said resin-forming ingredients in an atmosphere containing at least 50% of superheated steam.

The thermohardening synthetic resins employed in our invention are selected from the group which consists of urea-formaldehyde resin, melamine-formaldehyde resin and mixed melamine-formaldehyde urea formaldehyde resin.

The term "melamine" includes substituted melamines, such as alkylated melamine.

When the textile material treated in accordance with the present invention does not consist wholly of regenerated cellulose, it preferably contains more than about 80% by weight of regenerated cellulose. The regenerated cellulose is, preferably, viscose rayon. The invention is of particular value when the regenerated cellulose is spun viscose rayon.

It is well known that the insolubilisation substantially within and not between the fibres of a regenerated cellulose fabric without undue loss of resistance to abrasion, of a sufficient proportion of urea-formaldehyde resin, melamine-formaldehyde resin or mixed melamine-formaldehyde urea-formaldehyde resin will give crease-resistance, and even a degree of recovery from creasing comparable with that of high grade wool fabrics. In the case of urea-formaldehyde resin, an amount of, for example, 12 to 18% by weight of resin calculated upon the weight of dry fabric before treatment is suitable for this purpose in the case of most types of regenerated cellulose fabrics. Substantially 15%, for example, is a convenient amount. In the case of melamine-formaldehyde resins comparable results are obtained with considerably less resin, 7% for example being a convenient amount.

Useful effects can be obtained with smaller proportions

of any of the resins employed, i. e. stabilisation with reduced loss of resistance to abrasion.

It has been known that higher proportions of these resins would confer upon regenerated cellulose fabrics an even better crease-resistance, but because of the loss in the resistance of the fabric to abrasion which accompanies the treatment with such resins, the proportion that could usefully be insolubilised within the fibres has hitherto been limited, in commercial practice.

We have now found that much larger percentages of these resins can be insolubilised within the fibres of a textile fabric composed wholly or mainly of regenerated cellulose and thus the properties further improved, while maintaining satisfactory resistance to abrasion, or even obtaining a resistance to abrasion slightly better than that hitherto considered to be satisfactory, by carrying out the insolubilisation of the resin in the presence of not less than 50% of superheated steam. By effecting the insolubilisation in this way, it is possible, by correct choice of conditions, to obtain improved physical properties due to the larger percentage of resin, as well as improved resistance to abrasion compared with a fabric similarly treated but heated without added steam. By "larger percentages of resin" we mean over 20% by weight in the case of urea-formaldehyde resins and over 8% by weight in the case of melamine-formaldehyde resins or of mixed melamine-formaldehyde urea-formaldehyde resins, calculated upon the weight of the dry fabric before treatment.

In the customary process using urea-formaldehyde resin it has generally been considered necessary that the molecular proportion of formaldehyde to urea should not exceed about 1.6 to 1. It has been found that if the resin is made with substantially more than this proportion of formaldehyde, although it is fast to washing, and although the crease recovery properties of the fabric are greater than those of a fabric treated with resin formed from urea and formaldehyde in the proportions of about 1.6 to 1, the fabric is so tendered that it may have no commercial value. We have found that by using for the insolubilisation by heating an atmosphere containing at least 50% of superheated steam, in accordance with our invention, we may employ aqueous solutions of the urea-formaldehyde resin-forming ingredients wherein the molecular proportion of formaldehyde is at least 2 to 1, for example from 2½ to 1 to 4 to 1 and still obtain a fabric having a satisfactory resistance to abrasion.

Similarly, in using melamine-formaldehyde resin it has generally been considered necessary that the molecular proportion of formaldehyde to melamine should not exceed 3 to 1. It has been found that if the resin is made with substantially more than this proportion of formaldehyde, although it is fast to washing and the crease recovery properties of the treated fabric are greater than those of a fabric treated with resin made from melamine and formaldehyde in the molecular proportion 3 to 1, the fabric is so tendered that it may have no commercial value. We have found that by using for the insolubilisation by heating at atmosphere containing at least 50% of superheated steam in accordance with our invention, we may employ aqueous solutions of melamine-formaldehyde resin-forming ingredients wherein the molecular proportion of formaldehyde is greater than three to one, for example from 4 to 1 to 6 to 1 and still obtain a fabric having a satisfactory resistance to abrasion. Similar results are obtained when the resin is a mixed melamine-formaldehyde urea-formaldehyde resin wherein there are more than 3 molecular equivalents of formaldehyde for each molecular equivalent of melamine and more than 2 molecular equivalents of formaldehyde for each molecular equivalent of urea.

The temperature of drying should be below 100° C. and is preferably below 80° C., for example 40° C. to 60° C. During or immediately after drying, the impregnated fabric may be subjected to mechanical distortion

subsequently rendered permanent by the insolubilisation of the urea-formaldehyde resin; for example, it is possible to calender, to schreiner, to emboss or to produce glazed effects by friction or to pleat.

5 The temperature and time of heating to insolubilise the resin, when employing an atmosphere containing at least 50% of superheated steam according to the present invention, may be the same as that which would be employed without added steam or with the small proportions of steam which have hitherto been customary. This, as is known, exceeds 100° C. and preferably exceeds 120° C. Thus, temperatures between 130° and 180° C. are suitable, for example 150° C. The condensation may be carried out in the presence of the customary catalysts and in particular we may use a potentially acid catalyst, e. g. an ammonium salt or an amine salt.

In practicing the present invention, it is preferred to impregnate the textile material in the form of a fabric 20 with an aqueous solution containing a water-soluble crystallloid intermediate condensation product of the amino-formaldehyde resin and containing also an acidic catalyst, remove excess solution from the fabric, dry the fabric and then heat it in an atmosphere containing at 25 least 50% of superheated steam to complete the condensation, i. e. to insolubilise the resin.

The acidic catalyst may be an acid, a mixture of acids, a mixture of an acid and a salt, or, preferably, a potentially acid substance i. e. one which is capable of becoming acid (or more acid, e. g. a mixture of calcium chloride and boric acid) or of liberating acid during the treatment, for example aluminium chloride or, most suitably, an ammonium salt or an amine salt such as ammonium thiocyanate or ammonium dihydrogen phosphate.

When using catalysts which are weakly acid, the time and temperature are of the order of 3-5 minutes at 160-180° C. whereas with stronger acids (or substances capable of liberating stronger acids) the temperature may be reduced to 130-150° C.

40 A solution of intermediate condensation product of mixed melamine-formaldehyde and urea-formaldehyde resin of low molecular weight and capable of penetrating textile fibres, may be prepared in two ways; a melamine-formaldehyde intermediate condensation product and a urea-formaldehyde intermediate condensation product are prepared, mixed and suitably catalysed; or alternatively melamine and urea are mixed and then partially condensed with formaldehyde before catalysing. The 45 general technique of preparing a urea-formaldehyde intermediate condensation product may be in accordance with our British Patent No. 449,243.

The present invention may be carried out with mixtures of any melamine-formaldehyde and urea-formaldehyde intermediate condensation products capable of being insolubilised within the fibres by heating; for example methylol melamine and methylol urea, alkylated methylol melamine and methylol urea, methylol melamine and alkylated methylol urea, or alkylated methylol melamine 50 and alkylated methylol urea may be used.

60 The invention will be illustrated by but is not limited to the following examples.

Example 1.—100 gms. urea and 200 cc. of neutral 65 40% formaldehyde were mixed together and 9 cc. ammonium hydroxide (specific gravity 0.88) added. This mixture was then refluxed for 3 minutes and cooled to room temperature.

To 30 cc. of this refluxed mixture were added 10 cc. 70 of a 10% solution of ammonium dihydrogen phosphate and the volume made up to 100 cc. with water.

Two samples of spun viscose rayon fabric were impregnated in this solution, squeezed so as to contain about their own weight of liquor and dried at about 40° C.

One sample was then heated at atmospheric pressure

for 2 minutes at 150° C. in a hot air chamber without added steam. The other was heated at atmospheric pressure for 2 minutes at 150° C. in a hot air chamber containing a mixture of 16 parts of air and 84 parts of steam.

The two samples were then washed for 2 minutes at 90° C. in an aqueous washing medium containing 0.25% soap and 0.25% soda ash. They were then rinsed, dried and conditioned to normal moisture content.

When tested on the "ringwear testing machine" the sample heated without added steam wore through at 1148 cycles but the sample heated in the above-mentioned mixture of steam and air wore through only at 2162 cycles, an improvement of 88.3%.

*Example 2.*—The following Table II shows the effect of treating two fabrics according to the method described in Example 1 but using substantially 100% of superheated steam ("steam") as compared with fabrics similarly treated but in which the resin was insolubilised without added steam ("dry"), Fabric 1 was a viscose rayon fabric made from 75 denier filament warp and 30s cotton count spun rayon weft. Fabric 2 was a 100% viscose spun rayon fabric made from yarn spun to 30s cotton count.

Table II

| Fabric | Percent Steam | Ringwear  |     |       | Resin Content |       |
|--------|---------------|-----------|-----|-------|---------------|-------|
|        |               | Untreated | Dry | Steam | Dry           | Steam |
| 1      | 97            | 730       | 330 | 710   | 14.5          | 13.7  |
| 2      | 95            | 855       | 400 | 858   | 14.3          | 14.3  |

*Example 3.*—The following Table III shows that the improved wear resistance effect obtained by treating two fabrics according to the method described in Example 1 but using about 90% of superheated steam is substantially unaffected by washing.

Table III

| Fabric | Percent Steam | Percent Resin | Percent Improvement in Ringwear figure over dry insolubilisation |                 |     |       |
|--------|---------------|---------------|------------------------------------------------------------------|-----------------|-----|-------|
|        |               |               | Before Washing                                                   | After 10 washes | Dry | Steam |
| 3      | 92            | 9.8           | 110                                                              | 94              |     |       |
| 4      | 90            | 9.7           | 72                                                               | 93              |     |       |

Fabric 3 was a 100% viscose spun rayon dress fabric, the warp being made of staple viscose rayon fibres spun to 15s cotton count with alternate yarns of S and Z twist and the weft being made of staple viscose rayon fibres spun to 15s cotton count. Fabric 4 was a dress fabric made of a blend of 16% by weight of wool and 84% by weight of viscose spun rayon.

*Example 4.*—The following Table IV shows that there is less loss of resin on washing fabrics treated according to the method described in Example 1 but using atmospheres containing 90% of superheated steam and over, in which to insolubilise the resin ("steam"), as compared with fabrics in which the atmosphere used to insolubilise the resin contained no added steam ("dry").

Table IV

| Fabric | Steam content of oven, percent | Percentage loss on washing of resin originally present |       |     |       |
|--------|--------------------------------|--------------------------------------------------------|-------|-----|-------|
|        |                                | Dry                                                    | Steam | Dry | Steam |
| 3      | 92                             | 13                                                     | 9     | 7   | 6     |
| 4      | 90                             | 9                                                      | 7     | 5   | 4     |
| 5      | 96                             | 17                                                     | 11    | 8   | 7     |
| 6      | 96                             | 11                                                     | 8     | 6   | 5     |

Fabrics 3 and 4 were the same as in Example 3.

Fabrics 5 and 6 were viscose-acetate fabrics made from blended yarns containing 66½% staple viscose and 33½% staple acetate rayon.

*Example 5.*—22.7 kg. of urea were dissolved in 45.5 litres of 40% neutral formaldehyde and 1.5 litres of ammonia (0.88 specific gravity) added. This was mixed and allowed to stand overnight at room temperature, its final viscosity being 6.5 centipoises.

10 This concentrated reaction mixture was diluted with water until it contained 70% by volume of the concentrated reaction mixture and 3% of ammonium dihydrogen phosphate (calculated on the weight of the concentrated reaction mixture) added. A 100% viscose spun

15 rayon fabric and also a fabric composed of a blend of viscose and wool were each impregnated so as to retain 76% of its weight of the liquor, partially dried on steam heated cylinders and passed on to a stenter where it was dried to 36 inches wide. The fabrics were then each

20 divided into two parts; one part was heated at atmospheric pressure for 2.75 minutes at 160° C. without added steam and the other part was heated at atmospheric pressure for 2.75 minutes at 160° C. in the presence of 90% steam. Both parts were then washed in

25 open width in soda ash at 90° C. for 10 seconds, then in water at 90° C. for 10 seconds, then in water at 20° C. for 10 seconds, and then passed through a bath containing 1% of a sulphated fatty alcohol as a softener and dried on a stenter to 36 inches wide.

30 Other portions of the same fabrics were similarly prepared using diluted reaction mixtures containing 27.5%, 50% and 70% of the concentrated reaction mixture. The resin content (based on the weight of dry cellulose),

35 resistance to abrasion and dry recovery are shown in the following Tables V and VI. These tables also show that the recovery from creasing of fabrics in which the resin has been insolubilised in presence of superheated steam is substantially equal to that of fabrics in which the resin has been insolubilised in the absence of added

40 steam.

Table V

| 45 | 100% SPUN-VISCOSE RAYON FABRIC |      |                |       |          |       |                        |       |
|----|--------------------------------|------|----------------|-------|----------|-------|------------------------|-------|
|    | Strength of mixture, percent   |      | Resin, percent |       | Ringwear |       | Recovery from creasing |       |
|    |                                |      | Dry            | Steam | Dry      | Steam | Dry                    | Steam |
| 50 | 10.4                           | 9.8  | 942            | 1,754 | 3.0      | 2.8   | 2.9                    | 2.7   |
| 50 | 17.4                           | 16.4 | 560            | 1,481 | 3.1      | 2.9   | 2.8                    | 2.9   |
| 70 | 22.8                           | 21.1 | 494            | 1,049 | 3.4      | 3.2   | 3.3                    | 3.1   |

Table VI

55 FABRIC MADE FROM A BLEND OF 16% BY WEIGHT OF WOOL AND 84% BY WEIGHT OF VISCOSÉ STAPLE FIBRE

| 60   | Recovery from creasing       |      |               |       |          |       |     |       |
|------|------------------------------|------|---------------|-------|----------|-------|-----|-------|
|      | Strength of mixture, percent |      | Percent Resin |       | Ringwear |       |     |       |
|      |                              |      | Dry           | Steam | Dry      | Steam | Dry | Steam |
| 27.5 | 9.9                          | 9.8  | 670           | 1,780 | 3.4      | 3.3   | 3.4 | 3.2   |
| 50   | 16.1                         | 16.7 | 490           | 1,110 | 3.7      | 3.4   | 3.5 | 3.4   |
| 70   | 23.2                         | 23.3 | 380           | 1,050 | 3.7      | 3.6   | 3.6 | 3.5   |

Example 6.—100% viscose spun rayon and viscose spun rayon and wool mixture fabrics were treated as in Example 5 but with repeated impregnation with diluted reaction mixtures containing 50%, 60%, and 70% of the concentrated reaction mixture so as to obtain fabrics having higher resin contents than in Example 5. The resin content (based on the weight of dry fabric not containing resin), resistance to abrasion and dry recovery

75 are shown in the following tables VII and VIII.

100% VISCOSE SPUN RAYON FABRIC

| Strength of mixture, percent | Percent Resin |       | Ringwear |       | Recovery from creasing |      |       |      | Percent Steam | Percent Resin | Recovery from Creasing |      | Ringwear |  |  |  |
|------------------------------|---------------|-------|----------|-------|------------------------|------|-------|------|---------------|---------------|------------------------|------|----------|--|--|--|
|                              | Dry           | Steam | Dry      | Steam | Dry                    |      | Steam |      |               |               | Warp                   | Weft |          |  |  |  |
|                              |               |       |          |       | Warp                   | Weft | Warp  | Weft |               |               |                        |      |          |  |  |  |
| 50                           | 25.2          | 26.0  | 730      | 1,080 | 3.5                    | 3.2  | 3.6   | 3.2  |               | 10.5          | 3.3                    | 3.3  | 1,372    |  |  |  |
| 60                           | 33.9          | 30.1  | 789      | 1,240 | 3.6                    | 3.5  | 3.6   | 3.4  |               | 9.4           | 3.4                    | 3.4  | 1,561    |  |  |  |
| 70                           | 38.4          | 35.0  | 630      | 1,160 | 3.6                    | 3.4  | 3.7   | 3.4  |               | 9.4           | 3.2                    | 3.2  | 1,946    |  |  |  |
|                              |               |       |          |       |                        |      |       |      |               | 9.6           | 3.3                    | 3.1  | 1,974    |  |  |  |
|                              |               |       |          |       |                        |      |       |      |               | 8.6           | 3.3                    | 3.1  | 2,109    |  |  |  |
|                              |               |       |          |       |                        |      |       |      |               | 8.0           | 3.3                    | 3.2  | 2,683    |  |  |  |
|                              |               |       |          |       |                        |      |       |      |               | 8.2           | 3.4                    | 3.2  | 2,843    |  |  |  |

Table VIII

FABRIC MADE FROM A BLEND OF 16% BY WEIGHT OF WOOL AND 84% BY WEIGHT OF VISCOSE STAPLE FIBRE

| Strength of mixture, percent | Percent Resin |       | Ringwear |       | Recovery from creasing |      |       |      | Percent Steam | Percent Resin | Recovery from Creasing |      | Ringwear |  |  |  |
|------------------------------|---------------|-------|----------|-------|------------------------|------|-------|------|---------------|---------------|------------------------|------|----------|--|--|--|
|                              | Dry           | Steam | Dry      | Steam | Dry                    |      | Steam |      |               |               | Warp                   | Weft |          |  |  |  |
|                              |               |       |          |       | Warp                   | Weft | Warp  | Weft |               |               |                        |      |          |  |  |  |
| 50                           | 26.5          | 27.6  | 750      | 1,180 | 3.7                    | 3.7  | 3.7   | 3.6  |               | 26.5          | 3.7                    | 3.7  | 1,180    |  |  |  |
| 60                           | 33.8          | 31.5  | 680      | 1,280 | 3.8                    | 3.7  | 3.8   | 3.5  |               | 33.8          | 3.5                    | 3.5  | 1,280    |  |  |  |
| 70                           | 41.8          | 36.4  | 540      | 1,090 | 3.8                    | 3.8  | 3.8   | 3.8  |               | 41.8          | 3.8                    | 3.8  | 1,090    |  |  |  |

**Example 7.**—A ten percent solution in water of trimethylol-melamine intermediate condensation product (BT 314 sold by Beetle Products Co. Ltd.) was prepared and catalysed with five percent of ammonium dihydrogen phosphate on the weight of solid BT 314. This was used to treat different samples of a fabric of standard width made from a blend of 16% by weight of wool and 84% by weight of spun rayon. Each sample was impregnated so as to retain about 100 percent of its weight of the liquid, dried at a low temperature, and then heated at atmospheric pressure in an atmosphere containing superheated steam for 4 minutes at 145° C. The samples were then washed for 2 minutes in 1/4% soap and 1/4% soda ash solution at 90° C., rinsed in cold water and finally dried at the standard width. One sample, for comparison, treated in a similar way but was heated for 4 minutes at 145° C. in an atmosphere not containing steam.

The effect on abrasion resistance (as measured by the ringwear testing machine) of increasing the proportion of superheated steam is shown in the following Table IX.

Table IX

| Steam content, percent | Percent improvement of Ring Wear over dry-cured fabric |
|------------------------|--------------------------------------------------------|
| 18                     | 3                                                      |
| 20                     | 15                                                     |
| 35                     | 29                                                     |
| 50                     | 38                                                     |
| 70                     | 60                                                     |
| 95                     | 88                                                     |

It can be seen that as with fabrics treated with urea-formaldehyde resin, the abrasion resistance of fabrics treated with melamine-formaldehyde resin is improved by increasing the proportion of superheated steam in the atmosphere in which the resin is insolubilised.

**Example 8.**—Samples of a 100% viscose spun rayon fabric were treated as in Example 7 but each sample was impregnated so as to retain 80% instead of 100% of its weight of the liquid. In different samples the resin was insolubilised in atmospheres containing different proportions of superheated steam.

Table XI shows that in fabrics containing more than 8% of melamine-formaldehyde resin the resistance to abrasion, as measured by the ringwear testing machine, is improved by insolubilising the resin in atmospheres containing increasing proportions of superheated steam, and that recovery from creasing is unaltered.

15 **Example 9.**—Four concentrated reaction mixtures having different molecular proportions of formaldehyde to urea (referred to hereinafter as "formaldehyde ratios") were prepared by dissolving the urea in a 40% aqueous solution of formaldehyde, adding an aqueous solution of ammonia (specific gravity 0.88), mixing, and allowing to stand overnight at room temperature.

20 The amounts of the various ingredients in the mixtures were as follows:

Table XI

| Formaldehyde Ratio | Urea, Kg. | 40% Formaldehyde solution (Litres) | 0.88 S. G. Ammonia (Litres) |
|--------------------|-----------|------------------------------------|-----------------------------|
| 2:1                | 7.26      | 18.16                              | 0.726                       |
| 2.5:1              | 5.82      | 18.2                               | 0.654                       |
| 3:1                | 4.84      | 18.2                               | 0.604                       |
| 4:1                | 3.64      | 18.2                               | 0.545                       |

35 In addition, a mixture containing formaldehyde and urea in the molecular proportions of 1.6 to 1 was prepared as described in British Patent No. 449,243.

These concentrated reaction mixtures were diluted with water, catalysed by adding 5% of ammonium dihydrogen phosphate, calculated on the weight of dissolved urea and formaldehyde, and were used to impregnate samples of 100% viscose spun rayon fabrics as follows:

40 Each sample of fabric was impregnated with one of the above diluted and catalysed reaction mixtures so as to retain about 80% of its weight of the liquid, partially dried on steam heated cylinders and then passed on to a stenter where it was dried to the standard width. Some samples were heated at atmospheric pressure for 2 1/4 minutes at 160° C. in an atmosphere not containing added steam (hereinafter indicated in the tables by "D" after the formaldehyde ratio) and some samples were heated at atmospheric pressure for 2 1/4 minutes at 160° C. in an atmosphere containing 85-90% of superheated steam (hereinafter indicated in the tables by "S" after the 55 formaldehyde ratio). All samples were then washed in open width first in 2% sodium carbonate at 90° C. for 10 secs., then in water at 90° C. for 10 secs. and then in water at 20° C. for 10 secs.

45 They were then passed through a bath containing 1% of a sulphated fatty alcohol as a softener, and dried on a stenter to the standard width.

50 The effects obtained by treating these samples are shown in the following tables. The "laundry shrinkage" referred to in some of the tables was measured as follows:

55 The samples to be laundered were first measured and weighed. 40 litres of water at 40° C. and 75 gms. of soap were put into a washing machine using this quantity of water; the samples were then washed in the washing machine with agitation for 20 minutes. After centrifuging the samples were separated, rinsed in 40 litres of water at 40° C. for 5 minutes, and re-centrifuged. The samples were then shaken gently and pressed with a hot iron i.e. the iron is placed on the cloth for a few seconds without there being any horizontal movement of 60 the iron. After conditioning for approximately one hour,

75 the laundry shrinkage was measured.

the samples were re-measured and the shrinkage on warp and weft were calculated. A plus sign after a figure in the "Laundry shrinkage" column indicates that an extension has occurred.

Table XII shows the effect on the recovery from creasing abrasion resistance (as shown by the ringwear testing machine) and laundry shrinkage, of treating fabric with resin according to the method described above and using a reaction mixture having at least 2 molecular proportions of formaldehyde to 1 of urea and insolubilising the resin by heating in an atmosphere containing no added steam.

Table XII

100% VISCOSE SPUN RAYON FABRIC

| Formaldehyde Ratio | Percent Resin | Recovery from creasing |      | Ringwear |
|--------------------|---------------|------------------------|------|----------|
|                    |               | Warp                   | Weft |          |
| Untreated fabric   |               | 2.5                    | 2.4  | 1,870    |
| 1.6/1              | 11.7          | 3.0                    | 2.9  | 632      |
| 2/1                | 15.2          | 3.3                    | 3.3  | 342      |
| 2.5/1              | 16.5          | 3.5                    | 3.2  | 157      |
| 3/1                | 15.2          | 3.7                    | 3.4  | 150      |
| 4/1                | 17.5          | 3.8                    | 3.7  | 67       |

It will be seen that the crease-resistance is improved but that the abrasion resistance is drastically reduced by using greater formaldehyde ratios.

Table XIII shows the effect on the recovery from creasing, abrasion resistance (as shown by the ringwear testing machine) and laundry shrinkage of treating fabrics with resin according to the method described above and using a reaction mixture having at least 2 molecular proportions of formaldehyde to 1 of urea and insolubilising the resin by heating in an atmosphere containing superheated steam.

Table XIII

100% VISCOSE SPUN RAYON—FIRST FABRIC

| Formaldehyde Ratio | Percent Resin | Recovery from Creasing |      | Ring Wear | Laundry Shrinkage |      |
|--------------------|---------------|------------------------|------|-----------|-------------------|------|
|                    |               | Warp                   | Weft |           | Warp              | Weft |
| 1.6/1 D            | 15.5          | 3.1                    | 2.7  | 380       | 1.8               | 3.4  |
| 1.6/1 S            | 15.4          | 3.0                    | 2.7  | 1,080     |                   |      |
| 3/1 D              | 15.5          | 3.5                    | 3.2  | 120       |                   |      |
| 3/1 S              | 16.6          | 3.5                    | 3.2  | 333       | 0.5               | 0.9  |

100% VISCOSE SPUN RAYON—SECOND FABRIC

| 1.6/1 D | 15.5 | 3.3 | 2.9 | 220 |  |  |
|---------|------|-----|-----|-----|--|--|
| 1.6/1 S | 13.7 | 2.9 | 2.6 | 470 |  |  |
| 2/1 D   | 14.3 | 3.6 | 3.0 | 100 |  |  |
| 2/1 S   | 13.2 | 3.2 | 2.7 | 380 |  |  |
| 2.5/1 D | 13.7 | 3.6 | 3.2 | 90  |  |  |
| 2.5/1 S | 12.5 | 3.2 | 2.8 | 310 |  |  |
| 3/1 D   | 13.0 | 3.8 | 3.4 | 50  |  |  |
| 3/1 S   | 12.6 | 3.6 | 3.0 | 230 |  |  |
| 4/1 D   | 14.1 | 3.5 | 3.1 | 90  |  |  |
| 4/1 S   | 12.9 | 3.6 | 3.0 | 220 |  |  |

FABRIC CONSISTING OF 84% VISCOSE SPUN RAYON WITH 16% WOOL

| 1.6/1 D | 14.4 | 3.3 | 3.2 | 980   | 2.5 | 0.2 |
|---------|------|-----|-----|-------|-----|-----|
| S       | 13.5 | 3.5 | 3.3 | 2,100 | 2.9 | 0.2 |
| 2.0/1 D | 14.3 | 3.5 | 3.2 | 750   | 1.1 | 0.5 |
| S       | 12.2 | 3.5 | 3.2 | 1,840 | 1.8 | 0.9 |
| 2.5/1 D | 13.0 | 3.4 | 3.3 | 770   | 0.9 | 0.2 |
| S       | 12.9 | 3.6 | 3.4 | 1,320 | 1.3 | 0.9 |
| 3.0/1 D | 14.1 | 3.4 | 3.2 | 680   | 0.7 | 0.4 |
| S       | 12.6 | 3.7 | 3.5 | 1,200 | 0.3 | 0.4 |
| 4.0/1 D | 12.7 | 3.7 | 3.2 | 590   | 0.0 | 1.4 |
| S       | 11.8 | 3.6 | 3.4 | 1,010 | 1.1 | 1.1 |

It will be seen that increases in the formaldehyde ratio improve the recovery from creasing obtained by a given amount of resin and that when the resin is insolubilised in an atmosphere containing superheated steam the resistance to abrasion is substantially maintained as compared with the fabric treated with resin of 1.6/1 form-

aldehyde ratio and in which the resin is insolubilised in an atmosphere containing no added steam. It will also be seen that under the same conditions the laundry shrinkage is reduced.

Table XIV shows the effect on the laundry shrinkage resulting from repeated washings when the fabric is treated according to the method described above and using a reaction mixture having at least 2 molecular proportions of formaldehyde to 1 of urea and insolubilising the resin in an atmosphere containing superheated steam.

Table XIV

100% VISCOSE SPUN RAYON FABRIC

| Formaldehyde Ratio | Percent Resin | Number of Washings |      |      |      |      |      |      |      |
|--------------------|---------------|--------------------|------|------|------|------|------|------|------|
|                    |               | 2                  |      | 4    |      | 7    |      | 9    |      |
|                    |               | Warp               | Weft | Warp | Weft | Warp | Weft | Warp | Weft |
| 1.6/1 S            | 13.7          | 2.0                | 1.1  | 2.4  | 1.7  | 3.4  | 2.1  | 3.4  | 1.5  |
| 3/1 S              | 12.1          | 0.5                | 0.6  | 1.2  | 1.3  | 1.5  | 1.5  | 1.2  | 1.0  |

It will be seen that with fabric in which the resin is insolubilised in presence of superheated steam the shrinkage on repeated washing is less when the formaldehyde ratio is at least 2 to 1, specifically 3 to 1.

Table XV shows the effect on resistance to abrasion (as measured by the Ringwear testing machine) of treating the fabric according to the method described above and using a reaction mixture having a formaldehyde ratio of 3 to 1 and which has been diluted to 40% and insolubilising the resin by heating in an atmosphere containing increasing proportions of superheated steam.

Table XV

100% SPUN VISCOSE RAYON FABRIC

| Steam Content, percent | Percent improvement of Ringwear over dry-cured fabric |     |
|------------------------|-------------------------------------------------------|-----|
|                        | 0                                                     | 100 |
| 0                      | 0                                                     | 0   |
| 25                     | 121                                                   | 121 |
| 30                     | 130                                                   | 130 |
| 35                     | 150                                                   | 150 |
| 38                     | 233                                                   | 233 |
| 45                     | 235                                                   | 235 |
| 50                     | 332                                                   | 332 |
| 54                     | 302                                                   | 302 |
| 59                     | 277                                                   | 277 |
| 64                     | 288                                                   | 288 |
| 75                     | 321                                                   | 321 |
| 80                     | 371                                                   | 371 |
| 85                     | 409                                                   | 409 |
| 90                     | 416                                                   | 416 |
| 95                     | 435                                                   | 435 |

It will be seen that, as with fabric treated with resin having a formaldehyde ratio of 1.6 to 1, the resistance to abrasion is improved by insolubilising the resin in atmospheres containing high proportions of superheated steam when the formaldehyde ratio is 3 to 1.

We claim:

1. A process of giving increased abrasion resistance to a textile fabric containing at least 50% of regenerated cellulose by insolubilising in the fibers thereof, by heating, a resin selected from the group consisting of urea-formaldehyde wherein the molecular ratio of formaldehyde to urea is from 2:1 to 4:1, melamine-formaldehyde wherein the molecular ratio of formaldehyde to melamine is greater than 3:1 and up to 6:1, and a mixture of said urea-formaldehyde melamine-formaldehyde resins, which process comprises the steps of impregnating said fabric with an aqueous solution containing water-soluble ingredients for forming said resin, said solution also containing an acid catalyst for the resin formation, drying the fabric and heating it to produce said water-insoluble resin from said resin-forming ingredients in an atmos-

phere wherein at least 50% of said atmosphere is superheated steam.

2. A process of giving increased abrasion resistance to a textile fabric containing at least 50% of regenerated cellulose by insolubilising in the fibers thereof, by heating, a urea-formaldehyde resin wherein the molecular ratio of formaldehyde to urea is from 2:1 to 4:1, which process comprises the steps of impregnating said fabric with an aqueous solution containing water-soluble ingredients for forming said resin, said solution also containing an acid catalyst for the resin formation, drying the fabric and heating it to produce said water-insoluble urea-formaldehyde resin from said resin-forming ingredients in an atmosphere wherein at least 50% of said atmosphere is superheated steam.

3. A process of giving increased abrasion resistance to a textile fabric containing at least 50% of regenerated cellulose by insolubilising in the fibers thereof, by heating, a urea-formaldehyde resin wherein the molecular ratio of formaldehyde to urea is 3:1, which process comprises the steps of impregnating said fabric with an aqueous solution containing water-soluble ingredients for forming said resin, said solution also containing an acid catalyst for the resin formation, drying the fabric and heating it to produce said water-insoluble urea-formaldehyde resin from said resin-forming ingredients in an atmosphere wherein at least 50% of said atmosphere is superheated steam.

4. A process of giving increased abrasion resistance to a textile fabric containing at least 50% of regenerated cellulose by insolubilising in the fibers thereof, by heating, a melamine-formaldehyde resin wherein the molecular ratio of formaldehyde to melamine is greater than 3:1 and up to 6:1, which process comprises the steps of impregnating said fabric with an aqueous solution containing water-soluble ingredients for forming said resin, said solution also containing an acid catalyst for the resin formation, drying the fabric and heating it to produce said water-insoluble melamine-formaldehyde resin from said resin-forming ingredients in an atmosphere wherein at least 50% of said atmosphere is superheated steam.

5. A process of giving increased abrasion resistance to a textile fabric containing at least 50% of regenerated cellulose by insolubilising in the fibers thereof, by heating, a melamine formaldehyde resin wherein the molecular ratio of formaldehyde to melamine is 4:1, which process comprises the steps of impregnating said fabric with an aqueous solution containing water-soluble ingredients for forming said resin, said solution also containing an acid catalyst for the resin formation, drying the fabric and heating it to produce said water-insoluble melamine-formaldehyde resin from said resin-forming ingredients in an atmosphere wherein at least 50% of said atmosphere is superheated steam.

6. A process of giving increased abrasion resistance to a spun viscose rayon textile fabric by insolubilising in the fibers of said fabric, by heating, a resin selected from the group consisting of urea-formaldehyde wherein the molecular ratio of formaldehyde to urea is from 2:1 to 4:1, melamine-formaldehyde wherein the molecular ratio of formaldehyde to melamine is greater than 3:1 and up to 6:1, and a mixture of said urea-formaldehyde melamine-formaldehyde resins, which process comprises the step of impregnating said fabric with an aqueous solution containing a water-soluble crystalloidal intermediate condensation product of said resin, said solution also containing an acid catalyst for the resin formation, drying the fabric and heating it to produce said water-insoluble resin from said intermediate condensation product in an atmosphere wherein at least 50% of said atmosphere is superheated steam.

7. The process as defined in claim 2 wherein said urea-formaldehyde resin insolubilised in the fiber is at least 12%, calculated upon the weight of dry fabric before treatment.

8. The process as defined in claim 4 wherein the melamine-formaldehyde resin insolubilised in the fiber is at least 8%, calculated upon the weight of dry fabric before treatment.

9. A process of giving increased abrasion resistance to a textile fabric containing at least 50% of regenerated cellulose by insolubilising in the fibers thereof, by heating, a resin selected from the group consisting of urea-formaldehyde wherein the molecular ratio of formaldehyde to urea is from 2:1 to 4:1, melamine-formaldehyde wherein the molecular ratio of formaldehyde to melamine is greater than 3:1 and up to 6:1, and a mixture of said urea-formaldehyde melamine-formaldehyde resins, which process comprises the steps of impregnating said fabric with an aqueous solution containing water-soluble ingredients for forming said resin, said solution also containing an acid catalyst for the resin formation, drying the fabric and heating it to produce said water-insoluble resin from said resin-forming ingredients in an atmosphere consisting substantially wholly of superheated steam.

45 References Cited in the file of this patent

UNITED STATES PATENTS

|           |          |       |                |
|-----------|----------|-------|----------------|
| 2,088,227 | Battye   | ----- | July 27, 1937  |
| 2,093,651 | Widmer   | ----- | Sept. 21, 1937 |
| 2,190,672 | Meharg   | ----- | Feb. 20, 1940  |
| 2,299,786 | Battye   | ----- | Oct. 27, 1942  |
| 2,484,598 | Weisberg | ----- | Oct. 11, 1949  |
| 2,512,195 | Bener    | ----- | June 20, 1950  |
| 2,590,850 | Dungler  | ----- | Apr. 1, 1952   |